# EUROPEAN PATENT APPLICATION

(11) **EP 0 524 783 A1**
(43) Date of publication of application: **27.01.1993**
(21) Application number: 92306593.2
(22) Date of filing: 17.07.1992
(51) Int. Cl.: C10M 111/04, C10M 133/08, C10M 145/34, C10M 145/36, C10M 151/04, C10M 169/04

(54) **Use of lubricating oil compositions**

(30) Priority: 23.07.1991 GB 9115911; 23.07.1991 GB 9115912
(71) Applicant: OCEANFLOOR LIMITED, Southampton S04 6SZ (GB)
(72) Inventor: Cracknell, Robert Brian, BP Chemicals Limited, Hull HU12 8DS (GB)
(74) Representative: Preece, Michael

(57) **Abstract**

Use of a lubricating oil composition as an inlet-valve deposit inhibitor characterised in that the lubricating oil comprises a polyether of the formula

RX[(CₓH₂ₓO)ₙ(C_{y}H_{2y}O)ₚH]ₘ

wherein R is either an alkyl or alkylphenyl group having from 7 to 30 carbon atoms,
X is selected from 0,S or N, or RX together represent H,
x is an integer from 2 to 4,
y is an integer from 6 to 30,
m is 1 when X is O or S or when RX together represents H, or m is 2 when x is N, and
n and p are such that the polyether contains between 0 and 40% by weight of (C_{y}H_{2y}O) units and between 35 and 80% by weight of (CₓH₂ₓO) units is disclosed.

In particular, it is preferred to use a lubricating oil composition consisting essentially of the polyether, a synthetic lubricating oil and optionally a mineral oil.

In the preferred polyethers, the (CₓH₂ₓO) units comprise at least 50 mol % of oxypropylene units, preferably 100 mol %.

Preferred synthetic lubricating oils are polyalphaolefins and polyol esters.

## Description

The present invention relates to the use of lubricating oil compositions as inlet-valve deposit inhibitors, in particular the use of compositions comprising polyethers.

Multigrade lubricating oils for use in automotive engines comprise several components, in particular viscosity index improvers; these viscosity index improvers modify the viscometric properties of the lubricating oil; however, the problem with such additives is that they increase the deposits on the inlet valves of the engine and thereby impair the efficiency of the engine.

EP 246612 describes a lubricating oil based upon a mixture of mineral oil and a polyether. Whilst the description indicates that the polyether is freely soluble in the mineral oil, only compositions in which 5 to 60% by weight of the polyether is present are taught as being advantageous. The polyether is one having the general formula R[(CₙH₂ₙO)ₓ(CₘH₂ₘO)_{y}H]_{z} where R is a moiety derived from an organic starter, n is 2 to 4, m is 6 to 40, x and y are integers, z is 1 to 8 and the content of (CₘH₂ₘO) groups in the polyether is 15 to 60% by weight.

EP 0355977 discloses an industrial or automobile lubricating oil, for use, eg as automotive or industrial gear lubricants, two-stroke engine lubricants, which comprises (a) 0 to 40% by weight of mineral oil(s) and (b) 100 to 60% by weight of a polyether having the general formula RX[(CₓH₂ₓO)ₙ(C_{y}H_{2y}O)ₚH]ₘ wherein R is C₉ to C₃₀ alkyl or alkylphenyl, X is O, S or N, x is 2 to 4, y is 6 to 30, m is 1 or 2 and n and p are such that the polyether contains between 1 and 35% by weight of (C_{y}H_{2y}O) units and between 35 and 80% by weight of (CₓH₂ₓO) units. The polyether preferably has a molecular weight in the range 600 to 4000 and a viscosity in the range 32-460 mPa.s at 40°C.

However, the prior art does not disclose the use of such polyethers or compositions comprising such polyethers as inlet-valve deposit inhibitors. We have now found that specific polyethers can be used to improve inlet-valve deposit inhibition.

Thus, according to the present invention there is provided the use of a lubricating oil composition as an inlet-valve deposit inhibitor characterised in that the lubricating oil composition comprises a polyether of the formula

RX[(CₓH₂ₓO)ₙ(C_{y}H_{2y}O)ₚH]ₘ

wherein R is either an alkyl or alkylphenyl group having from 7 to 30 carbon atoms,
X is selected from 0,S or N, or RX together represent H,
x is an integer from 2 to 4,
y is an integer from 6 to 30,
m is 1 when X is O or S or when RX together represents H, or m is 2 when x is N, and
n and p are such that the polyether contains between 0 and 40% by weight of (C_{y}H_{2y}O) units and between 35 and 80% by weight of (CₓH₂ₓO) units.

The polyethers as defined above can be prepared as described in European Published Application EP 0355977.

The compositions of the present invention overcome the problems of the prior art by improving inlet valve deposit inhibition of automotive engines in which the compositions are used. Furthermore, the viscometric properties of the compositions are superior to those of the prior art compositions.

Considering the moiety R, this is suitably an alkyl or alkylphenyl group having from 7 to 30 carbon atoms. When R is an alkyl group it is preferably a C₁₀ to C₂₄ alkyl group, such as might be obtained from a corresponding fatty acid alcohol, thiol or amine. Most preferred are alkyl groups having 12 to 18 carbon atoms. In the case where R is alkylphenyl, R preferably has from 9 to 30 carbon atoms with phenyl groups substituted with one or more C₆ to C₁₂ alkyl groups being most preferred, preferably two, for example dinonyl phenol.

In addition to the moiety R and the group X the polyether is comprised of one or two independent oxyalkylene backbones of formula [(CₓH₂ₓO)ₙ(C_{y}H_{2y}0)ₚH]. Such backbones are created by alkoxylating a starter molecule of formula RX(H)ₘ with one or more alkylene oxides so that the backbone(s) formed comprise blocks of units of a given type. Alternatively the alkoxylation process can be carried out using a mixture of alkylene oxides in which case the backbones formed will comprise a random distribution of the units. For each of the two types of alkylene oxide, CₓH₂ₓ0 and C_{y}H_{2y}0, one or more different alkylene oxides can be used. The only constraint is that in the final polyether, the total number of units having the formula CₓH₂ₓ0 should comprise between 35 and 80, preferably between 45 and 65% by weight and the total number of units having the formula C_{y}H_{2y}O should comprise 0 to 40, preferably 1 to 30% by weight.

It is preferable that the units of formula (CₓH₂ₓ0) are mainly, ie greater than 50 mole %, comprised of oxypropylene (C₃H₆0) units. Most preferred are those polyethers where the CₓH₂ₓ0 groups are exclusively oxypropylene. As regards the (C_{y}H_{2y}0) units these are preferably such that y is in the range 12-20, for example when y = 16 wherein (C_{y}H_{2y}O) is derived from hexadecene-1-oxide.

The polyethers described above suitably have a weight molecular weight as measured by Gel Permeation Chromatography using polystyrene standards, in the range 400 to 4000, preferably 700 to 3000, more preferably from 800 to 2,500. They are also characterised by having a viscosity in the range 32 to 460 mPas at 40°C.

With the above constraints in mind it is most preferred that the polyether has the formula defined above with n being in the range 5 to 30 and p being in the range 1 to 4.

The lubricating oil compositions of the present invention may consist essentially of a polyether as defined hereinabove; optionally the lubricating oil composition may further comprise an animal, vegetable or mineral oil or a synthetic lubricating oil, preferably a mineral oil or a synthetic lubricating oil. A preferred combination is a polyether as defined hereinabove and a synthetic lubricating oil.

In a further aspect of the present invention there is provided the use of an industrial or automotive lubricating oil composition as an inlet valve deposit inhibitor characterised in that the composition consists essentially of
(a) from 5 to 95% by weight of one or more synthetic lubricating oils
(b) from 60 to 5% by weight of a polyether having the general formula

   RX[(CₓH₂ₓO)ₙ(C_{y}H_{2y}O)ₚH]ₘ

   wherein R is either an alkyl or alkylphenyl group having from 7 to 30 carbon atoms,
   X is selected from 0,S or N, or RX together represent H,
   x is an integer from 2 to 4,
   y is an integer from 6 to 30,
   m is 1 when X is O or S or when RX together represents H or m is 2 when x is N, and
   n and p are such that the polyether contains between 0 and 40% by weight of (C_{y}H_{2y}O) units and between 35 and 80% by weight of (CₓH₂ₓO) units and optionally
(c) a mineral oil

wherein the sum of (a) (b) and (c) does not exceed 100% by weight of the composition.

Suitable mineral oils include naphthenic and paraffinic oils.

Synthetic lubricating oils are synthesised by a chemical process as distinct from naturally occurring oils such as animal, vegetable or mineral oils. The term "synthetic lubricating oil" is a term well-known in the art. Suitable synthetic lubricating oils include polyesters such as pentaerythritol tetraesters, and polyol esters, diesters of dibasic acids or polyesters of polybasic acids such as dioctyl adipate, dioctyl sebacate and tridecyladipate, polymeric hydrocarbons such as liquid polyisobutenes and polyalphaolefins. The term synthetic lubricating oils will not encompass the polyethers as defined hereinabove.

The components of the lubricating oil compositions of the present invention must be compatible and the compositions must be storage stable, preferably for at least 1 year. Through routine testing the man skilled in the art would be able to formulate such compositions such that the above criteria are met.

Additives such as viscosity-index improvers, pour point depressants, detergent additives, anti-wear additives, extreme pressure additives, anti-oxidants, anti-corrosion and anti-foam agents etc may optionally be added to the compositions. Where additives are comprised in the lubricating oil compositions of the present invention, such additives must be compatible in the composition and the compositions must be storage stable, preferably for at least 1 year. It is not necessary for all the components of the compositions to be independently compatible with one another so long as they are compatible in the final composition. Through routine testing the man skilled in the art woud be able to formulate such compositions such that the above criteria are met.

Where the compositions of the present invention comprises polyether as defined hereinabove, and a synthetic lubricating oil, it is preferred that the ratio of polyether to synthetic lubricating oil is in the range 10:1 to 1:10, preferably 5:1 to 1:5. The sum of the polyether and synthetic lubricating oil should be at least 10%, by weight of total weight of the composition, preferably greater than 30%, more preferably greater than 50%.

The following Example illustrates the invention. Lubricating oil compositions were prepared by mixing together the following ingredients:

| | Example 1 (according to the invention) | Comparative Test 2 |
|---|---|---|
| | (Parts by Weight) | (Parts by Weight) |
| Hitec 164 Polyalphaolefin (ex Ethyl) | 50 | 50 |
| Hitec 166 Polyalphaolefin (ex Ethyl) | 25 | 25 |
| Priolube 3932 (Polyol Ester) (ex Unichema) | 10 | 25 |
| Oil Soluble Polyalkylene Glycol 1769 | 15 | |
| VI Improver (Olefin Graft Copolymer of Polymethylmethacrylate) | 10 | 8 |
| Additive Package (ADX 11414 ex Adibis) | 11 | 11 |

The compositions of Example 1, Comparative Test 2 and a standard monograde lubricant were all tested using the Ford Pinto Inlet Valve Merit Rating Engine Test. The test uses a standard fuel to assess the build up of deposits on the inlet valves derived from oil leaking down the valve stems. The inlet valves are rated for cleanliness (10 = clean) at the end of the test, and the average result determined.

### Example 3

The following lubricating oil composition was prepared:

| | Parts |
|---|---|
| 180 BHK (Hydrocracked Mineral Oil ex BP) | 45 |
| Priolube 3932 (Polyol Ester) (ex Unichema) | 45 |
| Oil Soluble Polyalkylene Glycol 1769 | 10 |
| VI Improver (Polymethylmethacrylate) | 4.8 |
| SG/CD Additive Package | 12.8 |

The composition of Example 3 was tested in the M102E Engine Cleanliness (Sludge and Wear) test. The multigrade CEC reference mineral oil RL 140 was used as a comparison. The results are given in Table I.

**Table I**

| | Example 3 | RL 140 |
|---|---|---|
| Engine Cleanliness (maximum rating 10) | 9.24 | 8.1 |
| Average Cam Wear (microns) | 57 | 70 |
| Average Tappet Wear (microns) | 3.6 | 2.7 |
| Average Inlet Valve Rating (maximum rating 10 per valve) | 8.63 | 8.5 |

Example 3 was also compared to a commercially available 10W-40 SG/CD lubricant based upon mineral oil and hydrocracked mineral oil. These results are given in Table II.

**Table II**

| | Example 3 | Reference Oil |
|---|---|---|
| Average Total Deposit per Valve (mg) | 115 | 271 |
| Average Tulip Deposit per Valve (mg) | 95 | 214 |
| Oil Consumption (g) | 300 | 350 |

The Oil Soluble Polyalkylene Glycol 1769 was prepared as described in EP 355 977 and comprises 14% by weight dinonyl phenol, 73.1% propylene oxide, 12.9% C₁₆ alpha olefin epoxide, the glycol has a viscosity at 100°C of 25.8 cSt, at 40°C of 191.0 cSt and a visocisty index of 172.

## Claims

1. The use of a lubricating oil composition as an inlet-valve deposit inhibitor characterised in that the lubricating oil composition comprises a polyether of the formula
RX[(CₓH₂ₓO)ₙ(C_{y}H_{2y}O)ₚH]ₘ
wherein R is either an alkyl or alkylphenyl group having from 7 to 30 carbon atoms,
X is selected from 0,S or N, or RX together represent H,
x is an integer from 2 to 4,
y is an integer from 6 to 30,
m is 1 when X is O or S or when RX together represents H, or m is 2 when x is N, and
n and p are such that the polyether contains between 0 and 40% by weight of (C_{y}H_{2y}O) units and between 35 and 80% by weight of (CₓH₂ₓO) units.

2. The use of a lubricating oil composition as claimed in claim 1 wherein R is a C₁₀ to C₂₄ alkyl group.

3. The use of a lubricating oil composition as claimed in claim 2 wherein R is a C₁₂ to C₁₈ alkyl group.

4. The use of a lubricating oil composition as claimed in any of the preceding claims wherein greater than 50 mol % of the (CₓH₂ₓO) units are oxypropylene units.

5. The use of a lubricating oil composition as claimed in any one of the preceding claims wherein y is an integer from 12 to 20.

6. The use of a lubricating oil composition as claimed in any one of the preceding claims wherein n is in the range 5 to 30 and p is in the range 1 to 4.

7. The use of a lubricating oil composition as an inlet valve deposit inhibitor characterised in that the composition consists essentially of:
(a) from 5 to 95% by weight of one or more synthetic lubricating oils
(b) from 60 to 5% by weight of a polyether having the general formula:
RX[(CₓH₂ₓO)ₙ(C_{y}H_{2y}O)ₚH]ₘ
wherein R is either an alkyl or alkylphenyl group having from 7 to 30 carbon atoms
X is selected from 0,S or N, or RX together represent H,
x is an integer from 2 to 4,
y is an integer from 6 to 30,
m is 1 when X is O or S or when RX together represent H, or m is 2 when x is N and
n and p are such that the polyether contains between 0 and 40% by weight of (C_{y}H_{2y}O) units and between 35 and 80% by weight of (CₓH₂ₓO) units and optionally
(c) a mineral oil
wherein the sum of (a) (b) and (c) does not exceed 100% by weight of the composition.

8. The use of a lubricating oil composition as claimed in claim 7 wherein the synthetic lubricating oil is a polyalphaolefin or a polyol ester.

9. The use of a lubricating oil composition as claimed in either claim 7 or claim 8 wherein the ratio of polyether to synthetic lubricating oil is in the range 5:1 to 1:5.

10. The use of a lubricating oil composition as claimed in any one of claims 7 to 9 wherein the sum of the polyether and the synthetic lubricating oil is greater than 10% by weight of the total weight of the composition preferably greater than 30%, for example 50%.
